

# UNITED STATES PATENT OFFICE.

CARL RUDOLF JAHN, OF SCHLEBUSCH, NEAR COLOGNE, GERMANY, ASSIGNOR TO THE FIRM OF SPRENGSTOFF A.-G. CARBONIT, OF HAMBURG, GERMANY.

## EXPLOSIVE SUBSTANCE.

1,253,691.

Specification of Letters Patent.

Patented Jan. 15, 1918.

No Drawing.

Application filed December 15, 1913. Serial No. 806,825.

To all whom it may concern:

Be it known that I, CARL RUDOLF JAHN, a subject of the Emperor of Germany, residing at Schlebusch, near Cologne-on-the-5 Rhine, in the German Empire, have invented certain new and useful Improvements in Explosive Substances, of which the following is a specification.

Hexanitro di-phenyl, the manufacture of 10 which is indicated in the *Reports of the German Society of Chemists*, B. 34,2174 by Ullmann and Bielecki, has been found, after tests which we have carried out, to be highly suitable as an explosive substance.

15 The hexanitro di-phenyl has the following formula of constitution:



It has the form of fine crystals of light 25 yellow color which have no detrimental action whatever on the skin, being neither corrosive nor coloring, in contradistinction to the majority of the nitro bodies hitherto in use, and in particular picric acid and hexanitro di-phenylamin, during the manu-30 facture of which the workmen show signs of poisoning and eczema, which as is well known renders its manufacture very difficult and dangerous.

A further advantage over the aforesaid 35 substances, resides in the fact that hexanitro di-phenyl has completely neutral properties, that is to say, does not form either with acids or alkalis any kind of salt, whereas picric acid forms ready explosive picrates, 40 as known when merely in contact with metals, and hexanitro di-phenylamin forms salts owing to its basic nature.

The hexanitro-di-phenyl is a perfectly 45 stable body which is absolutely fixed and the manipulation and treatment of which can take place without any danger.

The hexanitro di-phenyl is quite insoluble 50 in water, and slightly soluble in alcohol, acetone, benzol, and toluol. The temperature of vaporization of this body is above 320° C. while its melting point has been observed to be near 230° C.

In explosive power, hexanitro di-phenyl

is about 10% superior to the known hexanitro di-phenylamin. When tested in a 55 block of lead 50 grams of hexanitro di-phenyl produced a cavity of 1810 cubic centimeters, whereas hexanitro di-phenylamin produced a cavity of 1630 cubic centimeters. When compared with picric acid the difference in favor of hexanitro di-phenyl is still greater.

The properties above referred to make it highly suitable for use as an explosive substance by itself or in combination with other 60 compounds, for instance, as a filling for grenades, torpedoes and mines, as well as for the manufacture of primers and detonators, and also for all purposes for which 65 explosive substances are used.

70 Hexanitro di-phenyl is used in grenades, torpedoes and mines in a compressed state; it is readily susceptible to compression and under a pressure of 2500 atmospheres it attains a density of approximately 1.61. The 75 detonation is produced by a primer No. 8 with a filling of 2 grams of fulminate of mercury, or any other suitable primer may be used.

It is also suitable for use as an igniter, 80 as it readily transmits the initiated detonation to other explosive substances which are detonated with difficulty. For filling primers, hexanitro-di-phenyl is used in combination with fulminate of mercury or 85 with trinitrid of lead.

For compound explosive substances, hexanitro di-phenyl may be used in all cases 90 where other aromatic nitro bodies such as trinitrotoluol are used.

The explosive donarit, having the composition:

|                  |     |
|------------------|-----|
| Nitroglycerin    | 4%  |
| Trinitrotoluol   | 12% |
| Ammonium nitrate | 80% |
| Flour            | 4%  |

95

produces for example, when hexanitro di-phenyl is used instead of trinitrotoluol, a cavity greater by 20 cubic centimeters, when 100 tested in a block of lead.

What I claim and desire to secure by Letters Patent of the United States is:—

1. A mixture containing nitroglycerin, hexa-nitro-di-phenyl, ammonium nitrate and 105 flour.

2. A mixture containing 4% of nitroglycerin, 12% hexa-nitro-di-phenyl, 80% ammonium nitrate and 4% of flour.
3. An explosive mixture containing hexa-nitro-di-phenyl, an oxidizing salt, and a carbonaceous fuel.
4. An explosive mixture containing hexa-nitro-di-phenyl, an oxidizing salt, a carbonaceous fuel and a nitric aliphatic body.
- 10 5. An explosive mixture comprising hexa-

nitro-di-phenyl, an oxidizing salt capable of burning without leaving any material amount of ash, and an organic fuel.

In testimony whereof I affix my signature in presence of two witnesses.

CARL RUDOLF JAHN.

Witnesses:

LOUIS VANDORN,  
OSCAR DEPNER.